

## UNITED STATES PATENT OFFICE

2,087,990

## ALUMINUM-BASE ALLOYS

Joseph A. Nock, Jr., Tarentum, Pa., assignor to  
Aluminum Company of America, Pittsburgh,  
Pa., a corporation of Pennsylvania

No Drawing. Application August 10, 1936,  
Serial No. 95,179

20 Claims. (Cl. 148—21.1)

This invention relates generally to the heat treatable strong aluminum-base alloys containing copper, with or without the so-called hardeners or hardening elements manganese, chromium, zirconium, molybdenum, beryllium, boron, and titanium. More particularly the invention relates to aluminum-copper alloys containing silicon. One of the objects of the invention is to provide thermally treated articles of such alloys, 10 possessing greater improvement in one or another physical property than has heretofore been obtainable by thermal treatment. Another object of the invention is to provide articles composed of alloys of the type indicated, with improvement particularly in the direction of yield 15 strength in the artificially aged condition. Another object is to provide high hardness in articles composed of such alloys. A further object is to provide alloy articles which will have improved resistance to corrosion in the artificially aged condition. These and other objects I attain with these alloys by the addition thereto of a small amount of tin, not exceeding 0.1 per cent and preferably more than about 0.05 per cent. 20 In fact, I have found beneficial results to be obtained with as little as 0.005 per cent. The advantages of the invention are, however, obtained only when the alloy is free from magnesium, that is, when the metal is either totally absent or is 25 present only in amount so small as to be a mere impurity, not exceeding, say, about 0.1 per cent. 30

The alloys to which the invention herein claimed is directed are those containing copper 2.0 to 12.0 per cent and zinc 0.1 to 14.0 per cent, 35 with or without a total of 0.1 to 3.0 per cent of one or more of the so-called hardening elements mentioned above, the rest of the alloy being aluminum.

In amounts of about 0.15 to 15.0 per cent, tin 40 has been known as an alloying element which in aluminum-base alloys containing copper increases the fluidity and improves the machining and polishing characteristics of the alloy. Its use, however, has been generally discontinued, it 45 having been learned, as investigators have pointed out, that tin in the amounts heretofore used adversely affects the hot working characteristics of aluminum and aluminum-base alloys, diminishes the corrosion resistance of such materials, 50 and, generally, serves no useful function not more advantageously obtained with other alloying elements.

Contrary to the accepted opinion and trend of the art, I have discovered that certain small 55 amounts of tin are beneficial and desirable in

aluminum-copper alloys with or without one or more of the elements silicon, nickel, and zinc; any of which alloys may also contain one or more of the hardeners manganese, chromium, boron, molybdenum, zirconium, beryllium, and titanium. 5 In accordance with these discoveries and as a result of a series of experiments directed thereto, I have determined that tin is extremely beneficial and desirable when (1) the tin is present in amounts of 0.005 to 0.1 per cent by weight; (2) 10 the alloy contains copper; (3) the alloy contains no magnesium or contains that metal only in so small an amount as to constitute a mere impurity; (4) the alloy is artificially aged, that is to say, when the alloy is subjected to artificial 15 aging (preferably but not necessarily after high temperature heat treatment), say at a temperature between about 100° and 200° C.

The benefits of my invention appear to be due to the response of a peculiar internal alloy 20 structure to the artificial aging treatment. Aging phenomena in aluminum-base alloys are believed to be the result of the precipitation of an alloying element from a solid solution thereof in aluminum which is super-saturated with respect thereto. The precipitation is submicroscopic or on the border line between submicroscopic and microscopic. By careful methods, however, it is possible to prepare metal specimens which, under the action of an etching agent, 25 reveal a structure indicative of the artificially aged condition of the metal.

For example, a section of an artificially aged wrought aluminum alloy article composed of 4.0 per cent of copper without tin, etched with a mixture of hydrofluoric, hydrochloric and nitric acids, shows under a magnification of 500 diameters an aluminum matrix composed of contrasting grains having distinctly marked boundaries. 35 Particles of the constituent CuAl<sub>2</sub> are seen scattered through the matrix but substantially none are found in the grain boundaries. The same alloy containing 0.05 per cent of tin shows after the same artificial aging only slight grain contrast, the grain boundaries are distinctly less sharp, and they contain multitudes of small particles of CuAl<sub>2</sub>. According to the theories of submicroscopic precipitation, the differences in 40 structure noted in the tin-containing alloy indicate a more advanced stage of submicroscopic precipitation of CuAl<sub>2</sub>, in fact showing that the precipitation has advanced to a large extent beyond the submicroscopic to the microscopic stage. 45 This is evidenced by the particles of CuAl<sub>2</sub> in the 50

grain boundaries, resulting from coalescence of particles precipitated in submicroscopic size.

The foregoing enhanced aging phenomenon which occurs in the above described aluminum 5 alloys containing tin is particularly manifested in such alloys by the development, under the action of the artificial aging treatment, of certain unusual and distinctive properties now to be described.

10 When tin in amounts of 0.005 to 0.1 per cent is present in aluminum alloys containing 2.0 to 12.0 per cent of copper and free from magnesium, a relatively short artificial aging treatment will develop high hardness. Thus an aluminum alloy 15 casting containing 11.78 per cent of copper and 0.05 per cent of tin, heat treated for 16 hours at 515° C. and aged for 15 hours at 150° C., had a Brinell hardness of 122. The same alloy without tin, similarly heat treated and aged, had a Brinell hardness of only 107. Similarly, and under the same treatment, an alloy containing about 4.0 per cent of copper, about 10.0 per cent of silicon, and about 0.04 per cent of tin, developed a Brinell hardness of 124, while a similar 25 alloy not containing tin developed a Brinell hardness of only 106.

A further effect of the tin addition upon aging is particularly evidenced in certain specially valuable and preferred alloys. Under the influence 30 of aging treatments, aluminum alloys containing 2.0 to 6.5 per cent of copper, 0.005 to 0.1 per cent of tin, and substantially free from magnesium, developed yield strengths which are on the order 35 of 30 to 200 per cent greater than the yield strengths of similar alloys not containing tin. While the fundamental reasons for such increase in yield strength are obscure, the effect is very pronounced. For instance, a magnesium-free 40 aluminum-base alloy containing 4.0 per cent of copper and 0.05 per cent of tin was heat treated at 510° C. for 20 minutes, quenched to room temperature, and artificially aged for 18 hours at 150° C. This alloy had a yield strength of 43,000 45 pounds per square inch. A similar alloy, similarly treated but not containing tin, had a yield strength of only 20,200 pounds per square inch.

In addition to the effects described, my invention possesses another advantage. The artificial 50 aging of aluminum-base alloys containing copper in substantial amount usually results in a decreased resistance of the alloy to corrosion, but I have found that when these alloys, especially those of the preferred copper content (2.0 to 6.5 per cent as stated above) contain tin in the amount prescribed by my invention this detrimental result is considerably lessened by the enhanced aging effect. In particular the artificially 55 aged alloys show a marked decrease in propensity to undergo intercrystalline or intergranular corrosion, a type of corrosion which is more objectionable than the ordinary surface type because it is often not readily apparent and so is apt to escape observation until the corroded part 60 or article fails as a result of the internal weakening.

The aluminum-base alloys which are improved by the enhanced aging induced therein by the addition of small amounts of tin are those containing 70 2.0 to 12.0 per cent of copper, with or without certain other alloying elements which I have found to be useful in modifying the general properties of the alloy without masking or destroying the beneficial properties above noted. 75 Thus the aluminum-copper alloys may contain

0.1 to 3.0 per cent of a class of "hardening elements" which may be present, separately or together; each, however, not exceeding greatly the following limits: manganese 0.1 to 2.0 per cent, chromium 0.1 to 1.0 per cent, boron 0.1 to 0.5 per cent, molybdenum 0.1 to 1.0 per cent, zirconium 0.1 to 0.5 per cent, beryllium 0.1 to 2.0 per cent, and titanium 0.03 to 0.5 per cent. 5

I have determined that magnesium is a harmful addition to the alloys above described in that 10 its presence in substantial amounts destroys in large part the effects induced by the addition of small amounts of tin.

The preferred alloys are those in which one or all the above described properties are present 15 to a marked extent, especially the yield strength. These alloys, as above noted, contain 2.0 to 6.5 per cent of copper and 0.005 to 0.1 per cent of tin, 0.05 to 0.1 per cent being preferred, and they are characterized in the artificially aged condition 20 by a yield strength substantially higher than that of the same alloy devoid of tin. In their preferred form, these alloys may also contain 0.1 to 1.0 per cent, in total, of one or more of the 25 hardening elements above mentioned. For making castings of the preferred alloys that are to be used in the unworked condition the alloys may contain a total of 0.1 to 5.0 per cent of an element of the class consisting of zinc, nickel, and 30 silicon. When two or all three of the elements zinc, nickel, and silicon are present, the total should not exceed 5.0 per cent, the lower limits being nickel 0.05 per cent, zinc 0.05 per cent, and silicon 0.05 per cent. For making wrought articles, the same foregoing lower limits should 35 be observed, but where two or all three of the named elements are present, the upper limits should be, nickel 1.0 per cent, silicon 3.0 per cent, and zinc 5.0 per cent. For rolling or forging, the total amount of these elements should not exceed 40 3.0 or 4.0 per cent, but if the alloy is to be extruded a total of about 9.0 per cent is permissible. In general, for making cast unworked articles the lower limits for each element, when used alone, should be, silicon 0.1 per cent, nickel 0.1 per cent, 45 and zinc 0.1 per cent, and the upper limits should be, silicon 14.0 per cent, nickel 7.0 per cent, and zinc 14.0 per cent. Furthermore, if two or more of the elements are present in cast unworked articles, the lower limits should be, silicon 0.05 50 per cent, nickel 0.05 per cent, and zinc 0.05 per cent, the total amount of any two or more of the elements being 14.0 per cent, the total nickel content, however, not exceeding 7.0 per cent. 55

As specifically illustrating these alloys, an example of a wrought aluminum-base alloy without magnesium, containing about 4.4 per cent of copper, about 0.85 per cent of manganese, about 0.75 per cent of silicon, about 0.4 per cent of iron may be cited. Two alloys of this composition, 60 with and without the addition of 0.05 per cent of tin, were heat treated at 520° C. for 15 minutes, quenched in water, and subjected for 18 hours to an aging treatment at 143° C. The tin-free alloy had a tensile strength of 58,700 pounds per square 65 inch, a yield strength of 33,250 pounds per square inch, and an elongation of 16.8 per cent in two inches. The other alloy containing 0.05 per cent of tin had a tensile strength of 63,190 pounds per square inch, a yield strength of 46,250 pounds per square inch, and an elongation of 11.0 per cent in two inches. The effect of tin upon the yield strength and hardness of heat treated and artificially aged cast alloys is illustrated by the following examples. Aluminum-base alloys con- 70 75 75

taining copper 4.0 per cent, zinc 3.0 per cent; and copper 4.0 per cent, zinc 10.0 per cent; with and without the addition of 0.05 per cent of tin, were cast, heat treated at 504° C. for 20 hours, quenched in water, and aged at 154° C. for 16 hours. The yield strength and hardness values of these alloys that were obtained are as follows:

| 10 | Alloy composition |         |         | Yield strength<br>lbs. per sq.<br>inch | Brinell<br>hardness |
|----|-------------------|---------|---------|----------------------------------------|---------------------|
|    | Copper            | Zinc    | Tin     |                                        |                     |
| 15 | Percent           | Percent | Percent | 12,830                                 | 51.4                |
|    | 4.0               | 3.0     | 0.05    | 27,950                                 | 100.0               |
|    | 4.0               | 3.0     | 0.05    | 14,200                                 | 60.2                |
|    | 4.0               | 10.0    | 0.05    | 25,160                                 | 95.6                |
|    | 4.0               | 10.0    | 0.05    |                                        |                     |

The aging treatments and heat treatments to which the above mentioned alloys are subjected in order to develop their advantageous properties are the thermal treatments well known to the art. The heat treatment usually comprises heating the aluminum-copper alloys to above about 400° C. but below the temperature at which the lowest melting constituent of the alloy becomes molten, generally known as the point of incipient fusion. The alloy thus treated is, in the preferred practice, cooled rapidly, as by quenching in water or air, to room temperature. The artificial aging usually comprises heating the aluminum-copper alloy to temperatures of about 100 to 200° C. until the desired increase in properties is obtained. The artificial aging in the preferred practice of the invention is preceded by heat treatment, but the enhanced aging effect herein described and its general results may be developed to an advantageous extent by the artificial aging alone.

The aluminum-base alloys herein described and claimed are those containing at least 70.0 per cent of aluminum, which metal may contain impurities, such as amounts of iron up to about 1.5 per cent and, likewise, small amounts of silicon such as are known to occur in virgin aluminum.

The enhanced aging herein described as resulting from the addition of tin in the stated amount to magnesium-free aluminum alloys containing from 2.0 to 12.0 per cent of copper is obtained in both cast and wrought articles. In the case of castings of such alloys containing tin, I have found that heat treatment at elevated temperatures without artificial aging produces a higher ductility than is obtainable by heat treatment of a casting of the same alloy without the tin. This species of the invention I do not claim specifically herein but do so in my copending application Serial No. 606,755, filed April 21, 1932, and issued as United States Letters Patent 2,022,686, under date of December 3, 1935.

In the appended claims the term tensile property, or the like, is intended to include hardness as a property which can be favorably affected by the enhanced artificial aging produced by my invention. Also within the spirit of the appended claims the article may be an ingot or other body designed for further casting or for working, or it may be a cast or wrought article which is suitable for immediate use or sale or which may require some further operation to fit it for use or sale.

Articles and methods involving aluminum-copper alloys containing silicon; nickel; silicon and nickel; silicon and zinc; nickel and zinc; and silicon, nickel and zinc; and aluminum-copper alloys containing none of the elements silicon, nickel and zinc; are not claimed herein but are

claimed in my copending applications Serial Nos. 95,177, 95,178, 95,180, 95,181, 95,182, 95,193 and 606,756, respectively. This application is a continuation-in-part of my copending application Serial No. 606,756, filed April 21, 1932, now Patent 5 No. 2,062,321, dated Dec. 1, 1936.

I claim:

1. In a method of making an article of aluminum alloy, forming an article of a magnesium-free alloy containing copper 2.0 to 12.0 per cent, zinc 0.1 to 14.0 per cent, and tin 0.005 to 0.1 per cent, the remainder being essentially aluminum; and artificially aging the article whereby a tensile property of the alloy is improved over that of a like alloy free from tin. 15

2. In a method of making an article of aluminum alloy, forming an article of a magnesium-free alloy containing copper 2.0 to 6.5 per cent, zinc 0.1 to 5.0 per cent, and tin 0.005 to 0.1 per cent, the remainder being essentially aluminum; 20 and artificially aging the article whereby a tensile property of the alloy is improved over that of a like alloy free from tin.

3. In a method of making an article of aluminum alloy, forming an article of a magnesium-free alloy containing copper 2.0 to 12.0 per cent; zinc 0.1 to 14.0 per cent; tin 0.005 to 0.1 per cent; and at least one hardening element of the class consisting of manganese 0.1 to 2.0 per cent, chromium 0.1 to 1.0 per cent, boron 0.1 to 0.5 per cent, 30 molybdenum 0.1 to 1.0 per cent, zirconium 0.1 to 0.5 per cent, beryllium 0.1 to 2.0 per cent, and titanium 0.03 to 0.5 per cent, the total hardening content being 0.1 to 3.0 per cent, and the remainder being essentially aluminum; and artificially aging the article whereby a tensile property of the alloy is improved over that of a like alloy free from tin. 35

4. In a method of making an article of aluminum alloy, forming an article of a magnesium-free alloy containing copper 2.0 to 12.0 per cent, zinc 0.1 to 14.0 per cent, and tin 0.005 to 0.1 per cent, the remainder being essentially aluminum; and artificially aging the article between about 100° C. and 200° C. inclusive, whereby a tensile 45 property of the alloy is improved over that of a like alloy free from tin.

5. In a method of making an article of aluminum alloy, forming an article of a magnesium-free alloy containing copper 2.0 to 6.5 per cent, zinc 0.1 to 5.0 per cent, and tin 0.005 to 0.1 per cent, the remainder being essentially aluminum; and artificially aging the article between about 100° C. and 200° C. inclusive, whereby a tensile 55 property of the alloy is improved over that of a like alloy free from tin.

6. In a method of making an article of aluminum alloy, forming an article of a magnesium-free alloy containing copper 2.0 to 12.0 per cent; zinc 0.1 to 14.0 per cent; tin 0.005 to 0.1 per cent; and at least one hardening element of the class consisting of manganese 0.1 to 2.0 per cent, chromium 0.1 to 1.0 per cent, boron 0.1 to 0.5 per cent, molybdenum 0.1 to 1.0 per cent, zirconium 0.1 to 0.5 per cent, beryllium 0.1 to 2.0 per cent, and titanium 0.03 to 0.5 per cent, the total hardening content being 0.1 to 3.0 per cent, and the remainder being essentially aluminum; and artificially aging the article between about 100° C. and 200° C. inclusive, whereby a tensile 70 property of the alloy is improved over that of a like alloy free from tin.

7. In a method of making an article of aluminum alloy, forming an article of a magnesium-free alloy containing copper 2.0 to 12.0 per cent, 75

- zinc 0.1 to 14.0 per cent, and tin 0.005 to 0.1 per cent, the remainder being essentially aluminum; heat treating the article between about 400° C. and the temperature of incipient fusion; and 5 artificially aging the article between about 100° C. and 200° C. inclusive, whereby a tensile property of the alloy is improved over that of a like alloy free from tin.
8. In a method of making an article of aluminum alloy, forming an article of a magnesium-free alloy containing copper 2.0 to 12.0 per cent, zinc 0.1 to 14.0 per cent, and tin 0.05 to 0.1 per cent, the remainder being essentially aluminum; heat treating the article between about 400° C. 10 and the temperature of incipient fusion; and artificially aging the article between about 100° C. and 200° C. inclusive, whereby a tensile property of the alloy is improved over that of a like alloy free from tin.
- 15 13. An article of artificially aged aluminum alloy free from magnesium and containing copper 2.0 to 12.0 per cent, zinc 0.1 to 14.0 per cent, and tin 0.005 to 0.1 per cent, the remainder being essentially aluminum. 5
14. An article of artificially aged aluminum alloy free from magnesium and containing copper 2.0 to 12.0 per cent, zinc 0.1 to 14.0 per cent, and tin 0.005 to 0.1 per cent; and at least one element of the class of hardeners composed of 10 manganese, chromium, boron, molybdenum, zirconium, beryllium, and titanium, the total hardening content being 0.1 to 3.0 per cent, the remainder of the alloy being essentially aluminum.
- 15 15. An article of artificially aged aluminum alloy free from magnesium and containing copper 2.0 to 6.5 per cent, zinc 0.1 to 5.0 per cent, and tin 0.005 to 0.1 per cent, the remainder of the 15 alloy being essentially aluminum.
16. An article of artificially aged aluminum alloy free from magnesium and containing copper 2.0 to 6.5 per cent, zinc 0.1 to 5.0 per cent, tin 0.005 to 0.1 per cent; and at least one element of the class of hardeners composed of manganese, chromium, boron, molybdenum, zirconium, beryllium, and titanium, the total hardening content being 0.1 to 3.0 per cent, the remainder of the 20 alloy being essentially aluminum. 25
17. An article of thermally treated aluminum alloy free from magnesium and containing copper 2.0 to 12.0 per cent, zinc 0.1 to 14.0 per cent, and tin 0.005 to 0.1 per cent, the remainder being essentially aluminum; the alloy being characterized by a structure produced by heating the alloy to over 400° C. but below incipient fusion, cooling 30 the alloy, and thereafter artificially aging the 35 alloy. 35
18. An article of thermally treated aluminum alloy free from magnesium and containing copper 2.0 to 12.0 per cent, zinc 0.1 to 14.0 per cent, and tin 0.005 to 0.1 per cent; and at least one element of the class of hardeners composed of manganese, chromium, boron, molybdenum, zirconium, beryllium, and titanium, the total hardening content being 0.1 to 3.0 per cent, the remainder being essentially aluminum; the alloy being characterized by a structure produced by heating the alloy to over 400° C. but below incipient fusion, cooling the alloy, and thereafter artificially aging the 40 alloy. 45
19. An article of thermally treated aluminum alloy free from magnesium and containing copper 2.0 to 6.5 per cent, zinc 0.1 to 5.0 per cent, and tin 0.005 to 0.1 per cent, the remainder being essentially aluminum; the alloy being characterized by a structure produced by heating the alloy to over 400° C. but below incipient fusion, cooling the alloy, and thereafter artificially aging the 50 alloy. 55
20. An article of thermally treated aluminum alloy free from magnesium and containing copper 2.0 to 6.5 per cent, zinc 0.1 to 5.0 per cent, and tin 0.005 to 0.1 per cent; and at least one element of the class of hardeners composed of manganese, chromium, boron, molybdenum, zirconium, beryllium, and titanium, the total hardening content being 0.1 to 3.0 per cent, the remainder being essentially aluminum; the alloy being characterized by a structure produced by heating the alloy to over 400° C. but below incipient fusion, cooling the alloy, and thereafter artificially aging the 60 alloy. 65
- 60 60
- 65 65
- 70 70
- 75 75
- 80 80
- 85 85
- 90 90
- 95 95
- 100 100
- 105 105
- 110 110
- 115 115
- 120 120
- 125 125
- 130 130
- 135 135
- 140 140
- 145 145
- 150 150
- 155 155
- 160 160
- 165 165
- 170 170
- 175 175
- 180 180
- 185 185
- 190 190
- 195 195
- 200 200
- 205 205
- 210 210
- 215 215
- 220 220
- 225 225
- 230 230
- 235 235
- 240 240
- 245 245
- 250 250
- 255 255
- 260 260
- 265 265
- 270 270
- 275 275
- 280 280
- 285 285
- 290 290
- 295 295
- 300 300
- 305 305
- 310 310
- 315 315
- 320 320
- 325 325
- 330 330
- 335 335
- 340 340
- 345 345
- 350 350
- 355 355
- 360 360
- 365 365
- 370 370
- 375 375
- 380 380
- 385 385
- 390 390
- 395 395
- 400 400
- 405 405
- 410 410
- 415 415
- 420 420
- 425 425
- 430 430
- 435 435
- 440 440
- 445 445
- 450 450
- 455 455
- 460 460
- 465 465
- 470 470
- 475 475
- 480 480
- 485 485
- 490 490
- 495 495
- 500 500
- 505 505
- 510 510
- 515 515
- 520 520
- 525 525
- 530 530
- 535 535
- 540 540
- 545 545
- 550 550
- 555 555
- 560 560
- 565 565
- 570 570
- 575 575
- 580 580
- 585 585
- 590 590
- 595 595
- 600 600
- 605 605
- 610 610
- 615 615
- 620 620
- 625 625
- 630 630
- 635 635
- 640 640
- 645 645
- 650 650
- 655 655
- 660 660
- 665 665
- 670 670
- 675 675
- 680 680
- 685 685
- 690 690
- 695 695
- 700 700
- 705 705
- 710 710
- 715 715
- 720 720
- 725 725
- 730 730
- 735 735
- 740 740
- 745 745
- 750 750
- 755 755
- 760 760
- 765 765
- 770 770
- 775 775
- 780 780
- 785 785
- 790 790
- 795 795
- 800 800
- 805 805
- 810 810
- 815 815
- 820 820
- 825 825
- 830 830
- 835 835
- 840 840
- 845 845
- 850 850
- 855 855
- 860 860
- 865 865
- 870 870
- 875 875
- 880 880
- 885 885
- 890 890
- 895 895
- 900 900
- 905 905
- 910 910
- 915 915
- 920 920
- 925 925
- 930 930
- 935 935
- 940 940
- 945 945
- 950 950
- 955 955
- 960 960
- 965 965
- 970 970
- 975 975
- 980 980
- 985 985
- 990 990
- 995 995
- 1000 1000

CERTIFICATE OF CORRECTION.

Patent No. 2,087,990.

July 27, 1937.

JOSEPH A. NOCK, JR.

It is hereby certified that error appears in the printed specification of the above numbered patent requiring correction as follows: Page 3, second column, line 2, for the serial number "95,193" read 95,183; and that the said Letters Patent should be read with this correction therein that the same may conform to the record of the case in the Patent Office.

Signed and sealed this 21st day of September, A. D. 1937.

Henry Van Arsdale  
Acting Commissioner of Patents.

(Seal)